

## UNITED STATES PATENT OFFICE

2,058,574

## HYDROLYSIS OF ORGANIC ESTERS

Henry Dreyfus, London, England

No Drawing. Application April 26, 1933, Serial  
No. 668,068. In Great Britain May 6, 1932

8 Claims. (Cl. 8—20)

This invention relates to improvements in the hydrolysis of organic esters, and is more particularly concerned with processes for the saponification of cellulose acetate or other esters of cellulose.

The saponification of cellulose acetate filaments, threads, yarns, ribbons, fabrics or other materials, particularly when aqueous saponifying agents are employed, frequently results in a substantial loss in the tenacity of the yarn, and the principal object of the present invention is to modify the saponifying medium in such a way that loss in tenacity is decreased or eliminated. By applying the processes of the invention the tenacity of the yarns may even increase.

According to the present invention saponification is effected in the presence of an oil which is preferably contained in the saponifying medium itself. The oil may be of mineral, vegetable or animal character, and may be soluble or insoluble in the bath. Thus, for instance, soluble oils include sulphonated castor oil and other vegetable oils sufficiently sulphonated to be soluble in an aqueous bath.

The insoluble oils, for example hydrocarbon oils, such as paraffin or other fractions of petroleum or the aromatic or cyclo-aliphatic hydrocarbons and also vegetable oils, and particularly the non-drying oils, for example castor oil, olive oil, cocoanut oil, arachis oil, and semi-drying oils, for instance cotton seed oil and rape oil, and animal oils, e. g. whale oil, may be emulsified in an aqueous saponifying medium. Thus, for instance, they may be emulsified with the aid of soaps, sulphonated fats or oils or salts thereof, such as sulphonated castor oil, true sulphonic acids of aliphatic hydrocarbons or alcohols or of fatty acids or salts thereof, the salts and condensation products of amines, particularly amines containing hydroxy, carboxy or other hydrophilic groups, with resin and naphthenic acids and higher fatty acids e. g. ethanolamine and other alkylolamine soaps and amino-alkylamides of higher fatty acids and in the aromatic series naphthalene sulphonic acid compounds and particularly alkylated naphthalene sulphonic acids, such as propyl and isobutyl naphthalene sulphonic acids and the sulphonated condensation products of formaldehyde and naphthalene. The use of soaps whether of inorganic bases or of organic bases is particularly advantageous, since these exert a buffer action on the saponifying treatment in addition to being useful for emulsifying the insoluble oils.

The invention is not confined to the use of

aqueous saponifying media, since alcoholic or aqueous alcoholic media may also be employed. When alcoholic media are employed the saponifying agent may be present in a quantity less than that theoretically necessary to effect the desired degree of saponification, as is described in British Patent No. 125,153 and U. S. application S. Nos. 283,999 and 284,000 filed 8th June, 1928. The invention is however of the greatest advantage in relation to aqueous saponifying media, since these media are most potent in bringing about decrease in the tenacity of the threads.

The saponifying agent may be caustic soda, caustic potash or an alkali salt or other inorganic reagent, for example sodium silicate or trisodium phosphate. Such agents may be used in a proportion appropriate to bring about the desired degree of saponification.

The concentrations of saponifying agent employed may vary widely, depending upon the degree of saponification it is required to effect, the nature of the saponifying agent employed, the temperature of saponification and other factors. Thus relatively low concentrations of caustic soda or caustic potash, for example concentrations of .25% or .5% may be employed at normal or slightly elevated temperatures when materials are treated for comparatively long periods in hank or other package form or as fabrics, particularly when only a small degree of saponification is required, while when it is desired to treat filaments, yarns or similar materials during the course of their travel from one point to another, for example continuously with their production and/or with a stretching operation, higher concentrations and/or higher temperatures may be employed, for example concentrations of 3 to 5% or even up to 10-16% or more of caustic alkali at temperatures of 50 to 60 or 70° C. When such temperatures and concentrations are employed in connection with bath treatments, the time of contact of the materials with the bath will in general be relatively short, for example of the order of 10 or 30 seconds or a minute or thereabouts. The exact period will of course depend upon the degree of saponification desired. Saponification processes of this nature are very suitably carried out in a bath having a length of, for example, 80 to 100 feet, so that a rate of travel of the materials of 30 to 50 or even 100 metres per minute may be obtained. In the case of using high concentrations of caustic alkali it is desirable that buffer agents, as for example sodium acetate, sodium

chloride or soaps, should be present in order to minimize any deleterious action of the alkali upon the materials. The buffer agent employed should not be of such a nature or used in such quantities as to throw soluble oils out of solution or break down the emulsion, when an insoluble oil is employed. The use, in addition to the main saponifying agent, of another agent of less alkalinity e. g. lime in the form of a milk 5 or fine suspension or other agent, such as calcium carbonate, baryta, barium carbonate or the like enables considerably improved results to be obtained and also enables the concentration and total quantity of caustic soda or other saponifying agent to be reduced. This novel process is 10 described in my U. S. application S. No. 655,778 filed 8th February, 1933. When such substances are used, the considerations mentioned above in connection with buffer agents also arise. Thus 15 20 the substances employed should be chosen so that insoluble compounds are not formed, and for this reason the sulphonated and preferably highly sulphonated oils are of great value, either to act themselves as oils or as emulsifying agents 25 when insoluble oils are employed.

The concentrations of saponifying agents are referred to above particularly in relation to bath treatments. Where a padding treatment or other means of mechanical impregnation is employed high concentrations of saponifying agents 30 for example 15 to 20% or even more may in general be employed, since according to such methods of treatment the yarn is not in contact with large quantities of saponifying medium for any 35 length of time, and the method of application enables uniform distribution of the saponifying agent in the desired quantities to take place. The saponification may be conducted at about normal atmospheric temperature, or at somewhat 40 elevated temperatures, for example up to 60° C. or even more.

The saponifying medium employed may, if desired, contain a solvent or swelling agent for the materials under treatment, as for example any 45 of the substances mentioned below in connection with stretching. Alternatively the materials may be treated with solvents or swelling agents prior to saponification, or when saponification is carried out continuously with stretching or other 50 treatment in which the materials are obtained in a swollen condition, they may be treated while in such condition with the saponifying agent.

The actual saponification treatment may be effected in any suitable manner. For instance 55 the complete saponification may be effected in a bath treatment, in which case a long bath may be provided, or a comparatively short bath to which heat is applied, or the yarns may be simply padded or otherwise provided with a limited 60 quantity of the saponifying agent which is caused to act subsequent to the application thereof, for example by passages over heated drums in the manner described in U. S. Patents Nos. 1,884,622 and 1,884,623. The application of the saponifying 65 agent will usually be a uniform application over the whole length of the yarn, but the invention does not exclude the intermittent application of the saponifying agent as described in U. S. application S. No. 415,803 filed 21st December, 1929 for the purpose of obtaining fancy yarns 70 or fabrics. A further alternative consists in spraying the saponifying agent on to the yarns or fabrics in a uniform manner or applying the saponifying agent, for instance ammonia or an organic base, in the form of vapour, and in this

case also local effects may be produced e. g. by the application of resists or the use of stencils.

The degree of saponification effected in accordance with the present invention will vary with the object which it is desired to achieve. Relatively low saponification, such as a saponification resulting in a loss of weight of 2 to 5 or 10 or 15% on the weight of the cellulose acetate, may be applied with the object of conferring upon the material an affinity for cotton dyes or with the object of increasing the safe ironing point, though for this latter purpose a loss in weight of 10 to 20 or 30% or more is desirable. The invention also envisages a process in which the ester groups are completely or substantially 15 completely eliminated from the cellulose ester so as to produce a product which is wholly or almost wholly reconstituted cellulose and therefore resembles the artificial silks and other products made from viscose. In this connection reference 20 is made to U. S. application S. No. 655,773 filed 8th February, 1933 which is particularly concerned with the production of regenerated cellulose materials.

In order to shorten the time of contact of the 25 materials with the saponifying agent, and particularly in order to make use of the full length of the bath in bath treatments carried out while the materials are in motion, it may be advantageous to subject the materials to a previous treatment 30 in order to wet them out thoroughly. Methods of effecting this are described in U. S. application S. No. 655,773.

The process of the invention may be applied to the treatment of cellulose acetates or other 35 saponifiable esters of cellulose, for instance cellulose formate, propionate or butyrate, of all kinds. Esters of low, medium or high viscosity characteristics may be present in the treated yarns, 40 fabrics or other materials, for instance cellulose acetates having a viscosity of 5-10, 20-30 or 50-100 or 200 or more as measured by comparing the viscosity of a 6% solution in acetone against a standard of glycerine taken as 100. The yarns or other materials treated may consist wholly 45 of the cellulose ester or may contain other materials not deleteriously affected, as for instance natural or artificial cellulosic materials.

Furthermore the materials may be subjected 50 to a stretching operation before, during or after the saponifying treatment with a view to obtaining products of increased tenacity. This stretching of the yarns or other products may be carried out by any suitable process, as for example those specifically described in U. S. Patent No. 1,709,470 and U. S. application S. No. 378,684 filed 16th July, 1929, or the stretching in stages of U. S. application S. No. 573,424 filed 6th November, 1931. As described in U. S. application S. No. 602,844 filed 2nd April, 1932 considerable 60 economy and other advantages accrue by carrying out the stretching operation with the yarns, threads or the like in warp formation. Such a warp may be carried continuously through the stretching and saponifying operations. The 65 saponification of a number of threads in warp formation either as a separate operation or continuously with the stretching operation is described in detail in U. S. application S. No. 655,773 to which reference is made.

The saponification process of the present invention may also be applied to artificial filaments, threads and similar materials which have been intermittently stretched, for example according 70 to the processes described in U. S. applications S. 75

Nos. 573,422 filed 6th November, 1931 and 574,852 filed 13th November, 1931, and to the fabrics and other products containing such materials, as described in U. S. application S. No. 665,630 filed

5 April 12, 1933.

Instead of treating the materials during their travel from one point to another they may, if desired, be treated in the form of hanks or cakes or other packages, and such processes are particularly useful when applied to cakes of yarn obtained by collection in a centrifugal spinning box. In this connection reference is made broadly to U. S. application S. No. 655,773 in which details of suitable methods of carrying out such saponification are described.

The stretching may be facilitated by means of solvents or swelling agents for the cellulose acetate or other cellulose esters, or for cellulose in the case of stretching after a more or less complete saponification, for example aqueous solutions of thiocyanates, such as those of the alkalies, ammonium and alkaline earths, aqueous solutions of zinc chloride, acetic acid, formic acid, lactic acid, diacetone alcohol, acetone and the like; the ethers cyclic and non-cyclic, esters or ether-esters of olefine glycols and polyolefine glycols or of other polyhydric alcohols, for instance the mono- and di-methyl and ethyl ethers of ethylene glycol, the mono-methyl and ethyl ethers of propylene glycol, and the mono-ethyl ether of diethylene glycol, dioxane, methylene ethylene dioxide and their homologues and substitution products, glycol monoacetate, methyl glycol monoacetate, mono-, di- and tri-acetins, etc.; phenols, formaldehyde, acetaldehyde, dichloroethylene, methylene chloride and the like, or mixtures of these, or solvent mixtures. Such processes of stretching may be applied either to wet or to dry spun yarns, and low degrees of stretch e. g. 50-100% of the original length of the materials may be applied, though preferably the stretch is considerably greater, e. g. 400-500%. The yarn may be stretched after its formation either continuously or discontinuously with its production, and/or it may be stretched considerably during its formation. In dry spinning operations this involves a softening treatment during the dry spinning process so as to enable a substantial stretch to be applied to the materials, while in the case of wet spinning the nature of the coagulating bath or of the spinning solution may be such that a very considerable stretch may be imparted to the materials during their actual formation. Processes of this character are described in U. S. applications S. Nos. 402,785 filed 26th October, 1929, 418,414 filed 3rd January, 1930, 437,423 filed 20th March, 1930, 469,622 filed 21st July, 1930 and 601,043 filed 24th March, 1932. In general the stretching of the threads either during, continuously with or after their formation may be such as to impart to the threads an initial tenacity exceeding 1.5 grams per denier and preferably exceeding 2 or even 2.5 or more grams per denier.

Such a stretching of the materials and also the use of high viscosity esters may still further increase the dry tenacity of the saponified materials obtainable in accordance with the invention.

The following examples illustrate the invention but it is to be clearly understood that they do not limit it in any way:—

*Example 1*

75 A warp of cellulose acetate yarn, either

stretched or unstretched, is carried over a 2 or 3 bowl padding mangle in which it is impregnated with a saponifying solution of the following composition:—

7 parts of caustic soda  
3 parts of Turkey red oil  
90 parts of water

5

The nip of the mangle is adjusted so that the yarn retains about its own weight of liquor and the warp is carried directly from the padding mangle to a series of hollow steam heated rollers to effect saponification as described in U. S. Patents Nos. 1,884,622 and 1,884,623. Subsequently it is scoured to remove the oil and other substances.

*Example 2*

An olive oil emulsion containing a saponifying agent is made up in the following manner, the parts being by weight:—

2 parts of triethanolamine  
10 parts of oleic acid  
30 parts of olive oil

20

are thoroughly stirred until an approximately homogeneous mixture is obtained and then parts of water are added with constant stirring until a thick, smooth emulsion is obtained. 60 parts of olive oil are then added in small portions with constant stirring and then 50 parts of water in a similar manner. Stirring is continued until an even emulsion is obtained. The emulsion is then diluted about five times with a 4% solution of caustic soda preferably by first adding about an equal volume of caustic soda in relatively small amounts and then the remainder in gradually increasing quantities.

30

A number of cellulose acetate dry spun yarns in warp formation, as spun or after having been stretched to 400 or 500% of their original length, are led from a creel of bobbins through a reed and between nip rollers in a wetting out bath, and thence over another roller through a further reed and under a roller in a saponifying bath containing the emulsion described above at a temperature of 40-50° C. The length of the bath is about 90-100 feet, and at the further end of the bath the warp passes through a reed close to a feed roller and out of the bath to washing, drying and winding devices.

35

The speed of the yarns is about 40 metres per minute.

*Example 3*

An emulsion is prepared by stirring up about 1 part of light mineral oil with 20 parts of a 4% soap solution containing about ½-1% of caustic soda. A cellulose acetate yarn in hank or other form is then treated in the above emulsion for about 15 to 20 hours at 20 to 25° C. the ratio of the bath volume to the material treated being 20 to 40:1. When the desired degree of saponification is obtained, the yarn is washed to remove the oil and other substances, and then dried. A partially saponified yarn is thus obtained having an improved tenacity and extension and an affinity for cotton colors.

55

What I claim and desire to secure by Letters Patent is:—

1. Process for the saponification of artificial filaments, threads, yarns, ribbons, fabrics and other materials containing organic esters of cellulose, which comprises treating the materials with an alkaline saponifying medium throughout which is distributed an oil.

60

65

70

75

2. Process for the saponification of artificial filaments, threads, yarns, ribbons, fabrics and other materials containing cellulose acetate, which comprises treating the materials with an aqueous alkaline saponifying medium throughout which is distributed an oil.

3. Process for the saponification of artificial filaments, threads, yarns, ribbons, fabrics and other materials containing organic esters of cellulose, which comprises treating the materials with an aqueous saponifying medium containing a mineral alkali and a colloidally dispersed oil.

4. Process for the saponification of artificial filaments, threads, yarns, ribbons, fabrics and other materials containing cellulose acetate, which comprises treating the materials with an aqueous saponifying medium containing a mineral alkali and a colloidally dispersed oil.

5. Process for the saponification of artificial filaments, threads, yarns, ribbons, fabrics and other materials containing cellulose acetate, which comprises treating the materials at a temperature of at least 60° C. with an aqueous saponifying medium containing caustic soda in a concentration of from 3 to 5% throughout which is distributed an oil.

6. Process for the manufacture of strong artificial materials having an affinity for cotton dyes, which comprises saponifying filaments, threads,

yarns, ribbons and like materials containing organic esters of cellulose which have been stretched by at least 100% of their original length, by treatment with an aqueous medium containing a mineral alkali and a colloidal dispersion of an oil.

7. Process for the manufacture of strong artificial materials having an affinity for cotton dyes, which comprises saponifying filaments, threads, yarns, ribbons and like materials containing cellulose acetate which have been stretched by at least 100% of their original length, by treatment at a temperature of at least 60° C. with an aqueous saponifying medium containing caustic soda in a concentration of from 3 to 5% throughout which is distributed an oil.

8. Process for the manufacture of strong artificial materials having an affinity for cotton dyes, which comprises saponifying filaments, threads, yarns, ribbons and like materials containing cellulose acetate which have been stretched by at least 100% of their original length, by treatment at a temperature of at least 60° C. with an aqueous saponifying medium containing caustic soda in a concentration of from 3 to 5% throughout which is distributed an oil so as to effect a loss in weight of the order of 10% on the weight of the cellulose acetate.

HENRY DREYFUS.